

## UNITED STATES PATENT OFFICE

CAMILLE DREYFUS, OF NEW YORK, N. Y., AND HERBERT PLATT, OF CUMBERLAND, MARYLAND, ASSIGNORS TO CELANESE CORPORATION OF AMERICA, A CORPORATION OF DELAWARE

## TREATMENT OF FABRIC

No Drawing.

Application filed June 27, 1928. Serial No. 288,805.

This invention relates to the treatment of yarns or fabrics containing organic esters of cellulose and particularly cellulose acetate with a bath containing an alkaline agent, whereby the fabric may be treated with cotton dyes, and other of its properties improved.

An object of our invention is to treat yarns or fabrics containing organic esters of cellulose with an alkaline solution in such a manner that the yarn or fabric may be dyed with cotton dyes in a satisfactory manner.

Another object of our invention is to treat yarns or fabrics containing cellulose acetate with alkali solutions of sufficient concentration and in such manner that the same may be dyed with dischargeable colors, whereby discharge prints may be produced on such fabrics.

The discharge printing of fabric containing organic derivatives of cellulose and particularly cellulose acetate to produce light figures on dark backgrounds has heretofore offered serious difficulties. This is due to the fact that the dark colors, such as reds, blues and blacks that are available for the dyeing of cellulose acetate fabrics cannot be discharged by pastes containing ordinary color discharging agents. We have discovered that if fabrics containing cellulose acetate yarns are treated with an alkaline bath under the conditions set forth below, a fabric is produced which is capable of being dyed with dyes that may be discharged by printing pastes containing ordinary discharging agents. Moreover the fabric, when treated by our process, has further desirable properties, such as having its safe ironing point materially increased.

In accordance with our invention, we treat fabrics or yarns made of or containing organic esters of cellulose with a saponifying bath containing an alkaline solution of comparatively high concentration, preferably at low temperatures. The fabric may then be dyed with suitable dyes and if desired, the dyed fabric may then be printed with a discharge paste which contains a reducing agent, with or without colors, and the printed

fabric may then be steamed and further treated in any suitable manner.

The fabric to be treated by our invention may contain yarns of any suitable organic ester of cellulose such as cellulose acetate, cellulose formate, cellulose propionate or cellulose butyrate. The fabric may consist wholly of yarns made of one or more of these organic esters of cellulose, or it may be a mixed fabric containing yarns of these organic esters of cellulose and the yarns of other fibers. Examples of such mixed fabrics are mixed cellulose acetate and cotton, and mixed cellulose acetate and silk.

The saponifying bath may contain any suitable alkali and is preferably of comparatively high concentration. Of the alkalis that are suitable, sodium hydroxide, potassium hydroxide or ammonia may be mentioned. The concentration of the alkali solution is preferably from 5 to 20% by weight. We have found that the use of 10% caustic soda solution is suitable for causing the cellulose acetate fabric to take direct cotton dyes in a satisfactory manner. However, if it is also desired to increase the safe ironing temperature, a 20% caustic soda solution is preferred, since by the use of this solution the safe ironing temperature of a cellulose acetate fabric is increased from 220° C. to 260° C. However, no advantage from the dyeing point of view is obtained by using a caustic soda solution of greater than 10% concentration. The saponifying bath may also contain such assistants as alcohols, sodium acetate, etc.

The alkali solution may be applied to the fabric containing the organic esters of cellulose in any suitable manner. However, we prefer to apply the caustic soda to the fabric by padding the caustic solution onto the fabric and then permitting the same to stand for an appreciable length of time as will be described below. The temperature of treatment is preferably room temperature and should not exceed 35° C. for obtaining the best results.

The fabric after it has been treated with the saponifying bath, as above indicated, is capable of being dyed by dyestuffs that have an affinity for cellulose acetate but not for

cotton, such as are known as SRA dyes, and also by dyes that have an affinity for cotton but not for cellulose acetate, such as direct cotton dyes. The direct cotton colors available for dyeing this material are within all ranges of colors. These cotton dyes include blues, blacks and reds, which may be discharged by ordinary discharge printing pastes, and therefore discharge prints of dark backgrounds may be produced on this fabric, a result heretofore not attainable on fabrics containing cellulose acetate yarn.

The fabric, so treated and after having been dyed with direct cotton dyes, may be printed with a discharge paste which contains a reducing agent and which may or may not contain colors for printing the discharge portions. After printing with the discharge paste, the fabric is steamed and given other treatments as is well understood in the art.

The discharge paste may be applied in any suitable manner such as by means of engraved or embossed rolls, plates or blocks. The paste may also be applied through stencils by means of brushing or spraying. The discharge paste may contain any suitable reducing agent such as sodium hydrosulphite or zinc hydrosulphite or the substances known as "protolin" which is sulphoxalate of zinc formaldehyde. For obtaining a white background the sodium hydrosulphite or zinc hydrosulphite are preferred, whereas if a colored discharge is desired the protolin is preferred.

In order to further illustrate our invention the following specific example is given.

#### Example

A fabric consisting wholly of cellulose acetate yarn is padded through rolls that are covered with several thicknesses of heavy cotton lapping or other absorbent material, using a bath containing 100 parts of water and 10 parts of caustic soda. The caustic soda solution is at room temperature, and the fabric is given two runs through the pad. The nip on the pad is arranged so that the fabric picks up an amount of solution equal to its own weight. After the second run on the pad, the roll of fabric is allowed to run 15 minutes, and the solution is then very lightly extracted on the roll. The fabric with the remaining solution is allowed to stand overnight at room temperature. In carrying out this process, it is important to give due heed to the strength of the caustic soda solution and to the temperature of treatment, which should not exceed 35° C. Likewise it is of importance that the fabric should be batched with a minimum amount of tension and that the caustic soda solution should be allowed to remain on the fabric for a period comparable to that of overnight.

After standing overnight, the fabric is rinsed in water and is ready for dyeing. Of

the direct cotton dyes that may be used, the following are suitable for a light fastness equal to 75 hours in the fadeometer.

National solantine blue 4-GL  
Pontamine fast black CW (Color Index 539) 70  
Pontamine yellow CH (Color Index 365)  
Newport direct fast red F (Color Index 419)  
Amanil black BOL (American Aniline Prod. Co.) (Color Index No. 493)  
Newport light fast blue SFF 75  
Chlorantine fast blue RL (Ciba) (see Color Index Supp. page 31)  
Chlorantine fast blue 8-GL (Ciba) (see Color Index Supp. page 31). 80

If a diazotized and developed dye is desired, diaminogene extra (General Dyestuffs Corp.) (Color Index 317) or diazo fast green BL (General Dyestuffs Corp.) (Color Index No. 532) may be applied to the fabric and the same then diazotized and developed with beta naphthol.

For obtaining a navy color of good fastness to light (75 hours fadeometer) the following mixture may be used:

National solantine blue 4-GL  
Pontamine block CW (Color Index 539)  
Pontamine yellow CH (Color Index 365)  
Newport direct fast red F (Color Index 419). 95  
For a navy of modern fastness to light the following mixtures of dyes may be used:  
Diazine black H extra (Color Index No. 401)  
Chlorazol sky blue FF (Color Index No. 518)  
Pontamine yellow CH (Color Index No. 365)  
Newport fast scarlet 4-BA (Color Index 326). 100

For obtaining a black with good fastness to light pontamine black CW may be used.

If it is desired to obtain discharge printing effects, the fabric, after it has been dyed with any of the above mentioned dyestuffs, may be printed with a discharge paste containing:

| Parts               |     |
|---------------------|-----|
| Gum tragacanth 1/12 | 100 |
| Protolin            | 40  |
| Water               | 40  |

This paste is most suitable for obtaining colored discharges. If a white discharge is desired the protolin is replaced by a hydro-sulphite, such as formaldehyde hydrosulphite or sodium hydrosulphite and any suitable desired color is added to the paste. The fabric after printing is dried and steamed and then finished in any desired manner.

It is to be understood that the foregoing details are given merely by way of illustration and that many variations may be made therein without departing from the spirit 125 of this invention.

Having described our invention what we claim and desire to secure by Letters Patent is:

1. Method of treating fabric containing 120

organic esters of cellulose comprising padding the fabric with an alkaline solution corresponding to a caustic soda solution of a concentration of from 5 to 20% at a temperature below 35° C., in the absence of retarding agents, batching the fabric containing the alkaline solution for 8 to 14 hours and then removing the alkaline solution.

2. Method of treating fabric containing cellulose acetate comprising padding the fabric with an alkaline solution corresponding to a caustic soda solution of a concentration of from 5 to 20% at a temperature below 35° C., in the absence of retarding agents batching the fabric containing the alkaline solution for 8 to 14 hours and then removing the alkaline solution.

3. Method of treating fabric containing organic esters of cellulose comprising padding the fabric with an alkaline solution corresponding to a caustic soda solution of a concentration of about 15% at a temperature below 35° C., in the absence of retarding agents, batching the fabric containing the alkaline solution for 8 to 14 hours and then removing the alkaline solution.

4. Method of treating fabric containing cellulose acetate comprising padding the fabric with an alkaline solution corresponding to a caustic soda solution of a concentration of about 15% at a temperature below 35° C., in the absence of retarding agents, batching the fabric containing the alkaline solution for 8 to 14 hours and then removing the alkaline solution.

5. Method of altering the dyeing properties of a fabric containing yarns of cellulose acetate comprising padding the fabric with an alkaline solution corresponding to a caustic soda solution of 5 to 20% concentration at a temperature below 35° C. in such a manner that the fabric takes up substantially its own weight of alkaline solution, in the absence of retarding agents, batching the fabric containing the alkaline solution for 8 to 14 hours at said temperatures and then removing the alkaline solution.

6. Method of altering the dyeing properties of a fabric containing yarns of cellulose acetate comprising padding the fabric with an alkaline solution corresponding to a caustic soda solution of about 15% concentration at a temperature below 35° C. in such a manner that the fabric takes up substantially its own weight of alkaline solution, in the absence of retarding agents; batching the fabric containing the alkaline solution for 8 to 14 hours at said temperatures and then removing the alkaline solution.

60 In testimony whereof, we have hereunto subscribed our names.

CAMILLE DREYFUS.  
HERBERT PLATE.